# EUROPEAN PATENT APPLICATION

(11) **EP 2 824 204 A1**
(43) Date of publication of application: **14.01.2015**
(21) Application number: 13757070.1
(22) Date of filing: 01.03.2013
(51) Int. Cl.: C22C 38/00, B21D 22/20, C21D 9/00, C22C 38/60

(54) **STEEL SHEET FOR HOT PRESSING USE, PRESS-MOLDED ARTICLE, AND METHOD FOR PRODUCING PRESS-MOLDED ARTICLE**

(30) Priority: 09.03.2012 JP 2012053845
(71) Applicant: Kabushiki Kaisha Kobe Seiko Sho (Kobe Steel, Ltd.), Kobe-shi, Hyogo 651-8585 (JP)
(72) Inventor: MURAKAMI, Toshio, Kobe-shi Hyogo 651-2271 (JP); NAITOU, Junya, Kobe-shi Hyogo 651-2271 (JP); OKITA, Keisuke, kobe-shi Hyogo 651-2271 (JP); IKEDA, Shushi, Nagoya Aichi 450-0003 (JP)
(74) Representative: Müller-Boré & Partner Patentanwälte PartG mbB
(86) International application number: PCT/JP2013/055678
(87) International publication number: WO 2013/133165

(57) **Abstract**

A steel sheet for hot pressing use according to the present invention has a specified chemical component composition, wherein some of Ti-containing precipitates contained in the steel sheet, each of which having an equivalent circle diameter of 30 nm or less, have an average equivalent circle diameter of 6 nm or less, the precipitated Ti amount and the total Ti amount in the steel fulfill the relationship represented by formula (1) shown below, and the sum total of the fraction of bainite and the fraction of martensite in the metal microstructure is 80 area% or more. $Precipitated Ti amount \left(mass%\right) - 3.4 \left[N\right] \leq 0.5 \times \left[\left(total Ti amount \left(mass%\right)\right)-3.4\left[N\right]\right]$ (In the formula (1), [N] represents the content (mass%) of N in the steel.)

## Description

### [Technical Field]

The present invention relates to a steel sheet for hot pressing use used in manufacturing structural components of an automobile and suitable for hot press forming, a press-formed product obtained from such a steel sheet for hot pressing use, and a method for manufacturing the press-formed product, and relates more specifically to a steel sheet for hot pressing use that is useful in being applied to a hot press forming method securing a predetermined strength by being subjected to heat treatment simultaneously with impartation of the shape in forming a pre-heated steel sheet (blank) into a predetermined shape, a press-formed product, and a useful method for manufacturing such a press-formed product.

### [Background Art]

As one of the fuel economy improvement measures of an automobile triggered by global environment problems, weight reduction of the vehicle body is advancing, and it is necessary to high-strengthen a steel sheet used for an automobile as much as possible. On the other hand, when a steel sheet is high-strengthened, shape accuracy in press forming comes to deteriorate.

On this account, a hot press forming method has been employed for manufacturing components in which a steel sheet is heated to a predetermined temperature (for example, a temperature at which a state of an austenitic phase is achieved), the strength is lowered, the steel sheet is thereafter formed using a tool of a temperature (room temperature for example) lower than the steel sheet, thereby impartation of a shape and rapid heat treatment (quenching) utilizing the temperature difference of the both are executed simultaneously, and the strength after forming is secured. Also, such a hot-press forming method is referred to by various names such as a hot forming method, hot stamping method, hot stamp method, die quench method, and the like in addition to the hot press method.

Fig. 1 is a schematic explanatory drawing showing a tool configuration for executing hot press forming described above, 1 in the drawing is a punch, 2 is a die, 3 is a blank holder, 4 is a steel sheet (blank), BHF is a blank holding force, rp is punch shoulder radius, rd is die shoulder radius, and CL is punch/die clearance respectively. Also, out of these components, in the punch 1 and the die 2, passages 1a, 2a through which a cooling medium (water for example) can pass are formed inside of each, and it is configured that these members are cooled by making the cooling medium pass through these passages.

In hot press forming (hot deep drawing for example) using such a tool, forming is started in a state the steel sheet (blank) 4 is heated to a two-phase zone temperature (between Ac₁ transformation point and Ac₃ transformation point) or a single-phase zone temperature of Ac₃ transformation point or above and is softened. That is, in a state the steel sheet 4 in a high temperature state is sandwiched between the die 2 and the blank holder 3, the steel sheet 4 is pressed in to the inside of a hole of the die 2 by the punch 1, and is formed into a shape corresponding to the shape of the outer shape of the punch 1 while reducing the outside diameter of the steel sheet 4. Also, by cooling the punch 1 and the die 2 in parallel with forming, heat removal from the steel sheet 4 to the tools (the punch 1 and the die 2) is executed, holding and cooling are further executed at a forming bottom dead point (the temporal point the tip of the punch is positioned at the deepest point: the state shown in Fig. 1), and thereby quenching of the raw material is executed. By executing such a forming method, a formed product of 1,500 MPa class with excellent dimensional accuracy can be obtained, the forming load can be reduced compared with a case a component of a same strength class is cold-formed, and therefore less capacity of the press machine is needed.

As a steel sheet for hot pressing use widely used at present, one using 22Mn-B5 steel as a raw material is known. The steel sheet has the tensile strength of approximately 1,500 MPa and the elongation of approximately 6-8%, and is applied to a shock resistant member (a member not causing deformation as much as possible and not causing breakage in collision). However, application to a component requiring deformation such as an energy absorption member is difficult because elongation (ductility) is low.

As a steel sheet for hot pressing use exerting excellent elongation, technologies such as the patent literatures 1-4 for example have also been proposed. According to these technologies, the basic strength class of each steel sheet is adjusted by setting the carbon content in the steel sheet to various ranges, and elongation is improved by introducing ferrite with high deformability and reducing the average grain size of ferrite and martensite. Although these technologies are effective in improving elongation, they are still insufficient from the viewpoint of improving elongation matching the strength of the steel sheet. For example, those having 1,470 MPa or more of the tensile strength TS have the elongation EL of approximately 10.2% at the maximum, and further improvement is required.

On the other hand, even the formed product having a lower strength class compared to the hot stamp formed product, 980 MPa class or 1,180 MPa class of the tensile strength TS for example, having been studied until now has a problem in forming accuracy of cold press forming, and there are needs for low-strength hot press forming as an improvement measure therefor. At that time, it is necessary to largely improve energy absorption properties in the formed product.

Particularly, in recent years, development of the technology for differentiating the strength within a single component is proceeding. As such a technology, a technology has been proposed in which the portion that must be prevented from deforming has high strength (high strength side: shock resistant portion side), and the portion that needs energy absorption has low strength and high ductility (low strength side: energy absorption portion side). For example, in a passenger car of the middle class or above, there is a case that portions having both functions of shock resistant property and energy absorption property are provided within a component of a B-pillar and rear side member considering compatibility in a side collision and a rear collision (a function for protecting the counterpart side also when a small-sized car collides with). For the purpose of manufacturing such members, (a) a method of joining a steel sheet becoming of low strength even in being heated to a same temperature and tool-quenched to a normal steel sheet for hot pressing use (tailored weld blank: TWB), (b) a method for differentiating the strength for each region of a steel sheet by differentiating the cooling rate in the tool, (c) a method for differentiating the strength by differentiating the heating temperature for each region of a steel sheet, and the like have been proposed.

Although the tensile strength: 1,500 MPa class is achieved on the high strength side (shock resistant portion side) according to these technologies, the maximum tensile strength is 700 MPa and the elongation EL is approximately 17% on the low strength side (energy absorption portion side), and achievement of higher strength and higher ductility are required in order to further improve the energy absorption properties.

In the meantime, although automobile components are required to be joined mainly by spot welding, it is known that drop of the strength in the weld heat affected zone (HAZ) is extreme, and the strength of the welded joint drops (softening) (non-patent literature 1 for example).

### [Citation List]

### [Patent Literature]

[Patent Literature 1] JP-A 2010-065292
[Patent Literature 2] JP-A 2010-065293
[Patent Literature 3] JP-A 2010-065294
[Patent Literature 4] JP-A 2010-065295

### [Non-Patent Literature]

[Non-Patent Literature 1] Hirosue et al. "Nippon Steel Technical Report" No. 378, pp.15-20 (2003)

### [Summary of Invention]

### [Technical Problems]

The present invention has been developed in view of such circumstances as described above, and its object is to provide a steel sheet for hot pressing use capable of obtaining a press-formed product that can achieve the balance of high strength and elongation with a high level when uniform property is required within a formed product, capable of achieving the balance of high strength and elongation with a high level according to each region when regions corresponding to a shock resistant portion and an energy absorption portion are required within a single formed product, and useful in obtaining a press-formed product excellent in softening prevention property in a HAZ, a press-formed product exerting the properties described above, and a useful method for manufacturing such a press-formed product.

### [Solution to Problems]

The steel sheet for hot pressing use of the present invention which could achieve the object described above contains:
C: 0.15-0.5% (means mass%, hereinafter the same with respect to the chemical component composition);
Si: 0.2-3%;
Mn: 0.5-3%;
P: 0.05% or less (exclusive of 0%);
S: 0.05% or less (exclusive of 0%);
Al: 0.01-1%;
B: 0.0002-0.01%;
Ti: 3.4[N]+0.002% or more and 3.4[N]+0.1% or less ([N] expresses N content (mass%)), and
N: 0.001-0.01% respectively, with the remainder consisting of iron and inevitable impurities, in which
some of Ti-containing precipitates contained in the steel sheet, each of which having an equivalent circle diameter of 30 nm or less, have an average equivalent circle diameter of 6 nm or less, the precipitated Ti amount and the total Ti amount in the steel fulfill the relationship represented by formula (1) shown below, and the sum total of the fraction of bainite and the fraction of martensite in the metal microstructure is 80 area% or more. Also, "equivalent circle diameter" is the diameter of an imaginary circle having an area same to the size (area) of Ti containing precipitates (TiC for example) ("the average equivalent circle diameter" is the average value thereof). $Precipitated Ti amount \left(mass%\right) - 3.4 \left[N\right] \leq 0.5 \times \left[\left(total Ti amount \left(mass%\right)\right)-3.4\left[N\right]\right]$ (In the formula (1), [N] represents the content (mass%) of N in the steel.)

In the steel sheet for hot pressing use of the present invention, according to the necessity, it is also useful to contain, as other elements, (a) at least one element selected from the group consisting of V, Nb and Zr by 0.1% or less (exclusive of 0%) in total, (b) at least one element selected from the group consisting of Cu, Ni, Cr and Mo by 1% or less (exclusive of 0%) in total, (c) at least one element selected from the group consisting of Mg, Ca and REM by 0.01% or less (exclusive of 0%) in total, and the like, and the properties of the press-formed product is improved further according to the kind of the elements contained.

The method for manufacturing a press-formed product of the present invention which could achieve the object described above includes the steps of heating the steel sheet for hot pressing use as described above to a temperature of Ac₁ transformation point+20°C or above and Ac₃ transformation point-20°C or below, thereafter starting press-forming of the steel sheet, and holding the steel sheet at the bottom dead point and executing cooling to a temperature or below, the temperature being lower than the bainite transformation starting temperature Bs by 100°C, while securing the average cooling rate of 20°C/s or more within a tool.

In the press-formed product of the present invention, the metal microstructure within the pressed steel includes retained austenite: 3-20 area%, annealed martensite and/or annealed bainite: 30-87 area%, and martensite as quenched: 10-67 area%, some of Ti-containing precipitates contained in pressed steel, each of which having an equivalent circle diameter of 30 nm or less, have an average equivalent circle diameter of 10 nm or less, the precipitated Ti amount and the total Ti amount in the steel fulfill the relationship represented by the formula (1) shown below, and the balance of high strength and elongation can be achieved as the uniform property of a high level within the formed product. Also, the area ratio of annealed martensite and/or annealed bainite means the total area ratio of both microstructures when both microstructures are included, and means, when either one microstructure is included, the area ratio of the microstructure. $Precipitated Ti amount \left(mass%\right) - 3.4 \left[N\right] \leq 0.5 \times \left[\left(total Ti amount \left(mass%\right)\right)-3.4\left[N\right]\right]$ (In the formula (1), [N] represents the content (mass%) of N in the steel.)

On the other hand, another method for manufacturing a press-formed product of the present invention which could achieve the object described above includes the steps of using the steel sheet for hot pressing use as described above, dividing a heating region of the steel sheet into at least two regions, heating one region thereof to a temperature of Ac₃ transformation point or above and 950°C or below, heating another region to a temperature of Ac₁ transformation point+20°C or above and Ac₃ transformation point-20°C or below, thereafter starting press-forming of the both regions, and holding the both regions at the bottom dead point and executing cooling to a temperature of martensite transformation starting temperature Ms or below while securing the average cooling rate of 20°C/s or more within a tool.

Another press-formed product of the present invention is a press-formed product of a steel sheet having the chemical component composition as described above in which the pressed steel includes a first region whose metal microstructure includes retained austenite: 3 area% or more and 20 area% or less and martensite as quenched: 80 area% or more, and a second region whose metal microstructure includes retained austenite: 3-20 area%, annealed martensite and/or annealed bainite: 30-87 area%, and martensite as quenched: 10-67 area%, some of Ti-containing precipitates contained in steel of the second region, each of which having an equivalent circle diameter of 30 nm or less, have an average equivalent circle diameter of 10 nm or less, and the precipitated Ti amount and the total Ti amount in the steel fulfill the relationship represented by the formula (1) shown below. In such a press-formed product, the balance of high strength and elongation can be achieved with a high level according to each region, the regions corresponding to the shock resistant portion and the energy absorption portion are present within a single formed product, and softening prevention property of a HAZ in spot welding in the second region becomes excellent. $Precipitated Ti amount \left(mass%\right) - 3.4 \left[N\right] \leq 0.5 \times \left[\left(total Ti amount \left(mass%\right)\right)-3.4\left[N\right]\right]$ (In the formula (1), [N] represents the content (mass%) of N in the steel.)

### [Advantageous Effects of Invention]

According to the present invention, because a steel sheet is used in which the chemical component composition is strictly stipulated, the size of Ti-containing precipitates is controlled, the precipitation rate is controlled for Ti that does not form TiN, and the ratio of tempered hard phase (martensitic phase, bainitic phase and the like), hard phase (as-quenched martensite phase) and retained austenite phase is adjusted with respect to the metal microstructure, by hot-pressing the steel sheet under a predetermined condition, high strength-elongation balance of the press-formed product can be made a high level. Also, when hot-pressing is executed under different conditions in plural regions, the shock resistant portion and the energy absorption portion can be formed within a single formed product, the balance of high strength and elongation can be achieved with a high level for each portion, and softening prevention property in a HAZ becomes excellent.

### [Brief Description of Drawing]

[Fig. 1] Fig. 1 is a schematic explanatory drawing showing a tool configuration for executing hot press forming.

### [Description of Embodiments]

The present inventors carried out studies from various aspects in order to achieve such a steel sheet for hot pressing use that can obtain a press-formed product exhibiting excellent ductility (elongation) also while securing high strength after press-forming in manufacturing the press-formed product by heating a steel sheet to a predetermined temperature and thereafter executing hot press forming.

As a result of the studies, it was found out that, when the chemical component composition of the steel sheet for hot pressing use was strictly stipulated, the size of Ti-containing precipitates and precipitated Ti amount were controlled and the metal microstructure was made an appropriate one, by hot press forming of the steel sheet under a predetermined condition, a press-formed product in which retained austenite of a predetermined amount was secured after press forming and intrinsic ductility (residual ductility) was enhanced could be obtained, and the present invention was completed.

In the steel sheet for hot pressing use of the present invention, it is necessary to strictly stipulate the chemical component composition, and the reasons for limiting the range of each chemical component are as follows.

### [C: 0.15-0.5%]

C is an important element in achieving the balance of high strength and elongation of a case uniform properties are required within a formed product with a high level or in securing retained austenite particularly in the low strength/high ductility portion of a case the regions corresponding to a shock resistant portion and an energy absorption portion are required within a single formed product. Also, by concentration of C to austenite in heating of hot press forming, retained austenite can be formed after quenching. Also, C contributes to increase of the amount of martensite, and increases the strength. In order to exert such effects, C content should be 0.15% or more.

However, when C content becomes excessive and exceeds 0.5%, two phase zone heating range becomes narrow, and the balance of high strength and elongation of a case uniform properties are required within a formed product is not achieved with a high level, or it becomes hard to adjust the metal microstructure to that targeted particularly in the low strength/high ductility portion (a microstructure in which a predetermined amount of annealed martensite and/or annealed bainite is secured) of a case the regions corresponding to a shock resistant portion and an energy absorption portion are required within a single formed product. Preferable lower limit of C content is 0.17% or more (more preferably 0.20% or more), and more preferable upper limit is 0.45% or less (further more preferably 0.40% or less).

### [Si: 0.2-3%]

Si exerts an effect of forming retained austenite by suppressing that martensite is tempered during cooling of tool-quenching and cementite is formed, or that untransformed austenite is disintegrated. In order to exert such an effect, Si content should be 0.2% or more. Also, when Si content becomes excessive and exceeds 3%, ferrite is liable to be formed, formation of single-phase microstructure becomes hard in heating, and required fractions of bainite and martensite cannot be secured in a steel sheet for hot pressing use. Preferable lower limit of Si content is 0.5% or more (more preferably 1.0% or more), and preferable upper limit is 2.5% or less (more preferably 2.0% or less).

### [Mn: 0.5-3%]

Mn is an element effective in enhancing quenchability and suppressing formation of a microstructure (ferrite, pearlite, bainite and the like) other than martensite and retained austenite during cooling of tool-quenching. Also, Mn is an element stabilizing austenite, and is an element contributing to increase of retained austenite amount. In order to exert such effects, Mn should be contained by 0.5% or more. Although Mn content is preferable to be as much as possible when only properties are considered, because the cost of adding alloy increases, Mn content is made 3% or less. Preferable lower limit of Mn content is 0.7% or more (more preferably 1.0% or more), and preferable upper limit is 2.5% or less (more preferably 2.0% or less).

### [P: 0.05% or less (exclusive of 0%)]

Although P is an element inevitably included in steel, because P deteriorates ductility, P is preferable to be reduced as much as possible. However, because extreme reduction causes increase of the steel making cost and to make it 0% is difficult in manufacturing, P content is made 0.05% or less (exclusive of 0%). Preferable upper limit of P content is 0.045% or less (more preferably 0.040% or less).

### [S: 0.05% or less (exclusive of 0%)]

Similar to P, S is also an element inevitably included in steel, S deteriorates ductility, and therefore S is preferable to be reduced as much as possible. However, because extreme reduction causes increase of the steel making cost and to make it 0% is difficult in manufacturing, S content is made 0.05% or less (exclusive of 0%). Preferable upper limit of S content is 0.045% or less (more preferably 0.040% or less).

### [Al: 0.01-1%]

A1 is useful as a deoxidizing element, fixes solid-solution N present in steel as AlN, and is useful in improving ductility. In order to effectively exert such an effect, Al content should be 0.01% or more. However, when Al content becomes excessive and exceeds 1%, Al₂O₃ is formed excessively, and ductility is deteriorated. Also, preferable lower limit of Al content is 0.02% or more (more preferably 0.03% or more), and preferable upper limit is 0.8% or less (more preferably 0.6% or less).

### [B: 0.0002-0.01%]

B is an element contributing to prevention of formation of ferrite, pearlite and bainite during cooling after heating to a two-phase zone temperature of (Ac₁ transformation point - Ac₃ transformation point) because B has an action of suppressing ferrite transformation, pearlite transformation and bainite transformation on the high strength portion side, and to secure retained austenite. In order to exert such effects, B should be contained by 0.0002% or more, however, even when B is contained excessively exceeding 0.01%, the effects saturate. Preferable lower limit of B content is 0.0003% or more (more preferably 0.0005% or more), and preferable upper limit is 0.008% or less (more preferably 0.005% or less).

### [Ti: 3.4[N]+0.002% or more and 3.4[N]+0.1% or less: [N] expresses N content (mass%)]

Ti develops improvement effect of quenchability by fixing N and holding B in a solid solution state. In order to exert such an effect, it is important to contain Ti more than the stoichiometric ratio of Ti and N (3.4 times of N content) by 0.002% or more. Also, by making Ti added excessively relative to N present in a solid solution state within the hot stamp formed product and finely dispersing the precipitated compound, drop of the strength in the HAZ can be suppressed by precipitation strengthening caused by that Ti dissolved in welding the hot stamp formed product is formed as TiC and by the effect of delaying increase of the dislocation density and the like by the effect of preventing movement of dislocation by TiC. However, when Ti content becomes excessive to be more than 3.4[N]+0.1%, Ti-containing precipitates (TiN for example) formed is coarsened, and ductility of the steel sheet deteriorates. More preferable lower limit of Ti content is 3.4[N]+0.005% or more (further more preferably 3.4[N]+0.01% or more), and more preferable upper limit is 3.4[N]+0.09% or less (further more preferably 3.4[N]+0.08% or less).

### [N: 0.001-0.01%]

N is an element inevitably mixed in, and is preferable to be reduced as much as possible, however, because there is a limit in reducing N in an actual process, 0.001% is made the lower limit. Also, when N content becomes excessive, Ti-containing precipitates (TiN for example) formed is coarsened, these precipitates work as the fracture origin, ductility of the steel sheet is deteriorated, and therefore the upper limit is made 0.01%. More preferable upper limit of N content is 0.008% or less (further more preferably 0.006% or less).

The basic chemical composition in the steel sheet for hot pressing use of the present invention is as described above, and the remainder is iron and inevitable impurities other than P, S (O, H and the like for example). Further, in the steel sheet for hot pressing use of the present invention, according to the necessity, it is also useful to further contain (a) at least one element selected from the group consisting of V, Nb and Zr by 0.1% or less (exclusive of 0%) in total, (b) at least one element selected from the group consisting of Cu, Ni, Cr and Mo by 1% or less (exclusive of 0%) in total, (c) at least one element selected from the group consisting of Mg, Ca and REM by 0.01% or less (exclusive of 0%) in total, and the like, and the properties of the steel sheet for hot pressing use are improved further according to the kind of the element contained. Preferable range when these elements are contained and reasons for limiting the range are as follows.

### [At least one element selected from the group consisting of V, Nb and Zr by 0.1% or less (exclusive of 0%) in total]

V, Nb and Zr have effects of forming fine carbide and miniaturizing the microstructure by a pinning effect. In order to exert such effects, it is preferable to contain them by 0.001% or more in total. However, when the content of these elements becomes excessive, coarse carbide is formed and becomes a start point of breakage, and ductility is deteriorated adversely. Therefore, it is preferable to contain these elements by 0.1% or less in total. More preferable lower limit of the content of these elements in total is 0.005% or more (further more preferably 0.008% or more), and more preferable upper limit in total is 0.08% or less (further more preferably 0.06% or less).

### [At least one element selected from the group consisting of Cu, Ni, Cr and Mo: 1% or less (exclusive of 0%) in total]

Cu, Ni, Cr and Mo suppress ferrite transformation, pearlite transformation and bainite transformation, therefore prevent formation of ferrite, pearlite and bainite during cooling after heating, and act effectively in securing retained austenite. In order to exert such effects, it is preferable to contain them by 0.01% or more in total. Although the content is preferable to be as much as possible when only the properties are considered, because the cost for adding alloys increases, 1% or less in total is preferable. Also, because there is an action of largely increasing the strength of austenite, the load of hot rolling increases, manufacturing of the steel sheet becomes difficult, and therefore 1% or less is also preferable from the viewpoint of manufacturability. More preferable lower limit of these elements in total is 0.05% or more (further more preferably 0.06% or more), and more preferable upper limit in total is 0.5% or less (further more preferably 0.3% or less).

### [At least one element selected from the group consisting of Mg, Ca and REM by 0.01% or less (exclusive of 0%) in total]

Because these elements miniaturize inclusions, they act effectively in improving ductility. In order to exert such effects, it is preferable to contain them by 0.0001% or more in total. Although the content is preferable to be as much as possible when only the properties are considered, because the effects saturate, 0.01% or less in total is preferable. More preferable lower limit of these elements in total is 0.0002% or more (further more preferably 0.0005% or more), and more preferable upper limit in total is 0.005% or less (further more preferably 0.003% or less).

In the steel sheet for hot pressing use of the present invention, (A) some of Ti-containing precipitates contained in the steel sheet, each of which having an equivalent circle diameter of 30 nm or less, have an average equivalent circle diameter of 6 nm or less, (B) relationship of precipitated Ti amount (mass%)-3.4[N]≤0.5×[(total Ti amount (mass%))-3.4[N]] (the relationship of the formula (1) described above) is fulfilled, and (C) the metal microstructure contains at least either one of bainite and martensite, and the sum total of the fraction of bainite and the fraction of martensite is 80 area% or more, are also important requirements.

Control of Ti-containing precipitates and the formula (1) is for preventing softening of the HAZ and is the control required fundamentally for a formed product, however, variation of these values between before and after hot-press forming is small, and therefore it is necessary that they have already been controlled at the stage of before forming (the steel sheet for hot pressing use). By making Ti that is excessive relative to N in the steel before forming be present in a solid solution state or a fine state, Ti-containing precipitates can be maintained in the solid solution state or the fine state in heating of hot press forming. Thus, the amount of precipitated Ti in the press-formed product can be controlled to a predetermined amount or less, softening in the HAZ is prevented, and thereby the properties of the welded joint can be improved.

From such a viewpoint, it is necessary to disperse the Ti-containing precipitates finely, and, for the purpose, it is necessary that some of the Ti-containing precipitates contained in the steel sheet, each of which having an equivalent circle diameter of 30 nm or less, have an average equivalent circle diameter of 6 nm or less (the requirement of (A) described above). Also, the reason the equivalent circle diameter of the Ti-containing precipitates of the object is stipulated to be 30 nm or less is that it is necessary to control the Ti-containing precipitates and excluding TiN formed coarsely in the melting stage that does not affect microstructure change and properties thereafter. The size of the Ti-containing precipitates (the average equivalent circle diameter of the Ti-containing precipitates whose equivalent circle diameter is 30 nm or less) is preferably 5 nm or less, more preferably 3 nm or less. Further, the Ti-containing precipitates of the object of the present invention also include precipitates containing Ti such as TiVC, TiNbC, TiVCN, TiNbCN and the like in addition to TiC and TiN.

Further, as described below, although the average equivalent circle diameter of the Ti-containing precipitates whose equivalent circle diameter in the press-formed product is 30 nm or less is stipulated to be 10 nm or less, the same before forming (the steel sheet for hot pressing use) is stipulated to be 6 nm or less. The reason the size of the precipitates of the formed product is stipulated to be larger than that of the steel sheet is that Ti is present in the steel sheet as fine precipitates or in a solid solution state, and, when heating of 15 min or more at near 800°C is executed, the Ti-containing precipitates are slightly coarsened. In order to secure the properties as a formed product, it is necessary that the average equivalent circle diameter of the Ti-containing precipitates whose equivalent circle diameter is 30 nm or less is 10 nm or less. In order to achieve the precipitation state in the hot stamp formed product, it is necessary that the average equivalent circle diameter of fine precipitates of 30 nm or less is made 6 nm or less and that majority of Ti is present in a solid solution state in the stage of the steel sheet for hot stamp use.

Also, in the steel sheet for hot pressing use, it is necessary that, out of Ti, majority of Ti other than that used for precipitating and fixing N is present in the solid solution state or the fine state. For that purpose, it is necessary that the Ti amount present as the precipitates other than TiN (that is, precipitated Ti amount (mass%)-3.4[N]) is 0.5 times or below of the balance obtained by deducting Ti that forms TiN from total Ti (that is, 0.5×[(total Ti amount (mass%))-3.4[N]] or less) (the requirement of (B) described above). Precipitated Ti amount (mass%)-3.4[N] is preferably 0.4×[(total Ti amount (mass%))-3.4[N]] or less, more preferably 0.3×[(total Ti amount (mass%))-3.4[N]] or less.

Although control of the metal microstructure is intrinsically necessary for achieving desired strength-elongation balance in the formed product, the metal microstructure cannot be controlled only by the hot pressing condition, and it is necessary to control the microstructure of the raw material steel thereof (the steel sheet for hot pressing use) beforehand. In order to secure the proper amount of annealed martensite and annealed bainite which are fine and largely contributing to ductility in the press-formed product, it is necessary to make the sum total of the fraction of bainite and the fraction of martensite in the steel sheet for hot pressing use 80 area% or more. When the sum total of the fraction of bainite and the fraction of martensite is less than 80 area%, the fraction of annealed martensite and/or annealed bainite targeted in the formed steel sheet is hardly secured, and the amount of other microstructure (ferrite for example) increases to deteriorate the strength-elongation balance. The sum total of the fraction of bainite and the fraction of martensite is preferably 90 area% or more, more preferably 95 area% or more.

Further, in the steel sheet for hot pressing use of the present invention, although the remainder of the metal microstructure is not particularly limited, at least any of ferrite, pearlite or retained austenite can be cited for example.

The steel sheet (the steel sheet for hot pressing use) of the present invention as described above can be manufactured by that a billet obtained by melting steel having the chemical component composition as described above is subjected to hot rolling with heating temperature: 1,100°C or above (preferably 1,150°C or above) and 1,300°C or below (preferably 1,250°C or below) and the finish rolling temperature of 930°C or above (preferably 950°C or above) and 1,050°C or below (preferably 1,000°C or below), cooling (rapid cooling) is executed immediately thereafter to 450°C or below (preferably 400°C or below) with the average cooling rate of 20°C/s or more (preferably 30°C/s or more), and winding is executed at 100°C or above (preferably 150°C or above) and 450°C or below (preferably 400°C or below).

The method described above is for executing control so that (1) rolling is finished at a temperature range where dislocation introduced by hot rolling remains within austenite, (2) Ti-containing precipitates such as TiC and the like are formed finely on the dislocation by rapid cooling immediately thereafter, and (3) bainite transformation or martensite transformation is caused by rapid cooling and winding thereafter.

The steel sheet for hot pressing use having the chemical component composition, metal microstructure and Ti-precipitation state as described above may be used for manufacturing by a hot press forming as it is, and may be used for manufacturing by hot press forming after being subjected to cold rolling with the draft: 10-80% (preferably 20-70%) after pickling. Further, it is also possible to use the steel sheet for hot pressing use or the material obtained by cold rolling thereof for manufacturing by hot press forming after being subjected to such heat treatment of heating to 830°C or above (preferably 850°C or above and 900°C or below), rapid cooling thereafter to 450°C or below (preferably 400°C or below) at a cooling rate of 20°C/s or more (preferably 30°C/s or more), and thereafter holding at 450°C or below for 10 s or more and 1,000 s or less, or tempering at a temperature of 450°C or below. The steel sheet subjected to such cold rolling and heat treatment is also included in the steel sheet for hot pressing use of the present invention as far as the required properties are fulfilled. Also, the steel sheet for hot pressing use of the present invention may be subjected to plating containing at least one element out of Al, Zn, Mg and Si on the surface thereof (the surface of the base steel sheet).

By using the steel sheet for hot pressing use as described above, executing heating to a temperature of Ac₁ transformation point+20°C or above and Ac₃ transformation point-20°C or below, thereafter starting press-forming, and executing cooling to a temperature or below, the temperature being lower than the bainite transformation starting temperature Bs by 100°C, while securing the average cooling rate of 20°C/s or more within the tool during forming and after completion of forming, the press formed product having a single property (may be hereinafter referred to as "single region formed product") can have an optimum microstructure of low strength and high ductility. The reasons for stipulating each requirement in this forming method are as described below.

In order to form austenite between laths of martensite and bainite within the steel sheet and to form annealed martensite and annealed bainite excellent in ductility by annealing martensite and bainite, the heating temperature should be controlled to a predetermined range. When the heating temperature of the steel sheet is below Ac₁ transformation point+20°C, sufficient amount of austenite cannot be secured in heating, and a predetermined amount of retained austenite cannot be secured in the final microstructure (the microstructure of the formed product). Also, when the heating temperature of the steel sheet exceeds Ac₃ transformation point-20°C, the transformation amount to austenite increases excessively in heating, and a predetermined amount of annealed martensite and annealed bainite cannot be secured in the final microstructure (the microstructure of the formed product).

In order to make austenite formed in the heating step described above a desired microstructure while preventing formation of the microstructure such as ferrite or pearlite, it is necessary to hold the steel sheet at the bottom dead point and to properly control the average cooling rate and the cooling finishing temperature within the tool. From such a viewpoint, it is necessary to make the average cooling rate within the tool 20°C/s or more and to make the cooling finishing temperature a temperature or below, the temperature being lower than the bainite transformation starting temperature Bs by 100°C. The average cooling rate at that time is preferably 30°C/s or more (more preferably 40°C/s or more). By transforming austenite having been present in heating to bainite and martensite while preventing formation of the microstructure such as ferrite or pearlite by making the cooling finishing temperature a temperature or below, the temperature being lower than the bainite transformation starting temperature Bs by 100°C, fine austenite is made remain between the laths of bainite and martensite, and a predetermined amount of retained austenite is secured while securing bainite and martensite.

When the cooling finishing temperature becomes higher than the temperature that is lower than the bainite transformation starting temperature Bs by 100°C and the average cooling rate is less than 20°C/s, the microstructure such as ferrite, pearlite and the like is formed, a predetermined amount of retained austenite cannot be secured, and elongation (ductility) in the formed product deteriorates. Also, the cooling finishing temperature is not particularly limited as far as it is a temperature or below, the temperature being lower than Bs by 100°C, and can be the martensite transformation starting point Ms or below for example.

Although control of the average cooling rate basically becomes unnecessary at the stage the temperature becomes equal to or below the temperature lower than the bainite transformation starting temperature Bs by 100°C, cooling may be executed to the room temperature with the average cooling rate of 1°C/s or more and 100°C/s or less for example. Also, control of the average cooling rate within the tool while being held at the bottom dead point can be achieved by means such as (a) to control the temperature of the forming tool (the cooling medium shown in Fig. 1 above), and (b) to control the thermal conductivity of the tool.

In the press-formed product (single region formed product) manufactured by hot press forming as described above, the metal microstructure is formed of retained austenite: 3-20 area%, annealed martensite and/or annealed bainite: 30-87 area%, and martensite as quenched: 10-67 area%, and the balance of high strength and elongation can be achieved with a high level and as a uniform property within the formed product. The reasons for setting the range of each requirement (basic microstructure) in such a hot press-formed product are as described below.

Retained austenite has an effect of increasing the work hardening ratio (transformation induced plasticity) and improving ductility of the press-formed product by being transformed to martensite during plastic deformation. In order to exert such an effect, the fraction of retained austenite should be made 3 area% or more. Ductility becomes more excellent as the fraction of retained austenite is higher. In the composition used for a steel sheet for an automobile, retained austenite that can be secured is limited, and approximately 20 area% becomes the upper limit. Preferable lower limit of retained austenite is 5 area% or more (more preferably 7 area% or more).

By making the main microstructure annealed martensite and/or annealed bainite which is fine and has low dislocation density, ductility (elongation) of the press-formed product can be enhanced while securing a predetermined strength. From such a viewpoint, the fraction of annealed martensite and/or annealed bainite is made 30 area% or more. However, when this fraction exceeds 87 area%, the fraction of retained austenite becomes insufficient, and ductility (residual ductility) deteriorates. Preferable lower limit of annealed martensite and/or annealed bainite is 40 area% or more (more preferably 50 area% or more), and preferable upper limit is less than 80 area% (more preferably less than 70 area%).

Because martensite as quenched is a microstructure inferior in ductility, when much amount thereof is present, elongation is deteriorated, however, in order to achieve high strength of over 100 kg/mm² class in a microstructure with low matrix strength such as annealed martensite, it is necessary to secure a predetermined amount of martensite as quenched. From such a viewpoint, the fraction of martensite as quenched is made 10 area% or more. However, when the fraction of martensite as quenched increases excessively, strength increases excessively and elongation becomes insufficient, and therefore the fraction thereof should be 67 area% or less. Preferable lower limit of the fraction of martensite as quenched is 20 area% or more (more preferably 30 area% or more), and preferable upper limit is 60 area% or less (more preferably 50 area% or less).

There is no specific limit other than the microstructure described above, and ferrite, pearlite, bainite and the like may be included as the remainder microstructure, however, these microstructures are inferior in contribution to strength and contribution to ductility compared to other microstructures, and it is basically preferable not to be contained (it may also be 0 area%). However, up to 20 area% is allowable. The remainder microstructure is preferably 10 area% or less, more preferably 5 area% or less.

In the press-formed product (single region formed product) described above, some of Ti-containing precipitates contained in the steel sheet, each of which having an equivalent circle diameter of 30 nm or less, have an average equivalent circle diameter of 10 nm or less. By fulfilling such a requirement, a press-formed product capable of achieving the balance of high strength and elongation with a high level can be obtained. The average equivalent circle diameter of Ti-containing precipitates having 30 nm or less equivalent circle diameter is preferably 8 nm or less, more preferably 6 nm or less.

Also, in the press-formed product (single region formed product), the amount of Ti present as the precipitates other than TiN (precipitated Ti amount (mass%)-3.4[N]) is 0.5 times or less of Ti of the balance obtained by deducting Ti that forms TiN from total Ti (that is 0.5×[(total Ti amount (mass%))-3.4[N]] or less). By fulfilling such a requirement, because Ti dissolved at the time of welding is finely precipitated in the HAZ and existing fine Ti-containing precipitates suppresses restoration of dislocation and the like, softening in the HAZ is prevented, and weldability becomes excellent. Precipitated Ti amount (mass%)-3.4[N] is preferably 0.4×[(total Ti amount (mass%))-3.4[N]] or less, more preferably 0.3×[(total Ti amount (mass%))-3.4[N]] or less.

When the steel sheet for hot pressing use of the present invention is used, by properly adjusting the press forming condition (heating temperature and cooling rate), the properties such as strength, elongation and the like of the press-formed product can be controlled, the press-formed product with high ductility (residual ductility) is obtained, and therefore application to a portion (energy absorption member for example) to which it has been difficult to apply conventional press-formed products becomes also possible which is very useful in expanding the application range of the press-formed product. Also, not only the single region formed product described above, a press-formed product exerting strength-ductility balance according to each region (may be hereinafter referred to as "plural region formed product") is obtained when the heating temperature and the condition of each region in forming are properly controlled and the microstructure of each region is adjusted in manufacturing the press-formed product by press forming of a steel sheet using a press-forming tool.

The plural region formed product can be manufactured as described above using the steel sheet for hot pressing use of the present invention by dividing a heating region of the steel sheet into at least two regions, heating one region thereof (hereinafter referred to as the first region) to a temperature of Ac₃ transformation point or above and 950°C or below, heating another region (hereinafter referred to as the second region) to a temperature of Ac₁ transformation point+20°C or above and Ac₃ transformation point-20°C or below, thereafter starting press forming of both of the first and second regions, and being held at the bottom dead point in both of the first and second regions and executing cooling to a temperature of martensite transformation starting temperature Ms or below while securing the average cooling rate of 20°C/s or more within a tool.

According to the method described above, by dividing the heating region of the steel sheet into at least two regions (high strength side region and low strength side region) and controlling the manufacturing condition according to each region, such a press-formed product that strength-ductility balance according to each region is exerted is obtained. The second region out of two regions corresponds to the low strength side region, and the manufacturing condition, microstructure and properties in this region is basically same to those of the single region formed product described above. Below, the manufacturing condition for forming the other first region (corresponding to the high strength side region) will be described. Also, in executing this manufacturing method, it is required to form regions with different heating temperature by a single steel sheet, however, by using an existing heating furnace (for example, far infrared furnace, electric furnace+shield), controlling while making the boundary section of the temperature 50 mm or less is possible.

### (Manufacturing condition of the first region/high strength side region)

In order to properly adjust the microstructure of the press-formed product, it is necessary to control the heating temperature to a predetermined range. By properly controlling this heating temperature, transformation to a microstructure mainly of martensite is caused while securing a predetermined amount of retained austenite in the cooling step after heating, and a desired microstructure can be achieved within the range of the final hot press-formed product. When the steel sheet heating temperature in this region is below Ac₃ transformation point, a sufficient amount of austenite cannot be obtained in heating, and a predetermined amount of retained austenite cannot be secured in the final microstructure (the microstructure of the formed product). Also, when the heating temperature of the steel sheet exceeds 950°C, the grain size of austenite becomes large in heating, martensite transformation starting temperature (Ms point) and martensite transformation finishing temperature (Mf point) rise, retained austenite cannot be secured in quenching, and excellent formability is not achieved. The heating temperature of the steel sheet is preferably Ac₃ transformation point+50°C or above and 930°C or below.

In order to make austenite formed in the heating step described above a desired microstructure while preventing formation of the microstructure such as ferrite or pearlite, it is necessary to be held at the bottom dead point and to properly control the average cooling rate and the cooling finishing temperature within the tool. From such a viewpoint, the average cooling rate should be 20°C/s or more and the cooling finishing temperature should be martensite transformation starting temperature (Ms point) or below. The average cooling rate at that time is preferably 30°C/s or more (more preferably 40°C/s or more). By transforming austenite having been present in heating to martensite while preventing formation of the microstructure such as ferrite or pearlite by making the cooling finishing temperature the martensite transformation starting temperature (Ms point) or below, martensite is secured. Specifically, the cooling finishing temperature is 400°C or below, preferably 300°C or below.

In the press-formed product obtained by such a method, the metal microstructure, precipitates and the like are different between the first region and the second region. In the first region, the metal microstructure is of retained austenite: 3-20 area% (the action and effect of retained austenite are same to the above), and martensite as quenched: 80 area% or more. In the second region, the metal microstructure and Ti state (the average equivalent circle diameter of Ti-containing precipitates, the value of the precipitated Ti amount (mass%)-3.4[N], and the like) same to those of the single region formed product described above are fulfilled.

By making the main microstructure of the first region martensite with high strength containing a predetermined amount of retained austenite, ductility and high strength in a specific region in the press-formed product can be secured. From such a viewpoint, the area fraction of martensite as quenched should be 80 area% or more. The fraction of martensite as quenched is preferably 85 area% or more (more preferably 90 area% or more). Also, as the microstructure in the first region, ferrite, pearlite, bainite and the like may be included in a part thereof.

Although the effect of the present invention will be shown below more specifically by examples, the examples described below do not limit the present invention, and any of the design alterations judging from the purposes described above and below is to be included in the technical range of the present invention.

### [Examples]

### [Example 1]

Steel (steel Nos. 1-32) having the chemical component composition shown in Tables 1, 2 below was molten in vacuum, was made a slab for experiment, was thereafter made a steel sheet by hot rolling, was thereafter cooled, and was subjected to treatment that simulates winding (sheet thickness: 3.0 mm). The winding simulated treatment method included cooling to the winding temperature, putting the sample thereafter into a furnace heated to the winding temperature, holding for 30 min, and cooling in the furnace. The manufacturing condition for the steel sheet at that time is shown in Table 3 below. Also, Ac₁ transformation point, Ac₃ transformation point, Ms point, and Bs point in Tables 1, 2 were obtained using the formulae (2)-(5) below (refer to "The Physical Metallurgy of Steels", Leslie, Maruzen Company, Limited (1985) for example). Also, the treatment (1)-(3) shown in the remarks column in Table 3 expresses that each treatment (rolling, cooling, alloying) shown below was executed.${Ac}_{1} transformation point \left(°C\right) = 723 + 29.1 \times \left[Si\right] - 10.7 \times \left[Mn\right] + 16.9 \times \left[Cr\right] - 16.9 \times \left[Ni\right]$ $\begin{matrix} {Ac}_{1} transformation point \left(°C\right) \\ = 910 - 203 \times {\left[C\right]}^{1 / 2} + 44.7 \times \left[Si\right] - 30 \times \left[Mn\right] + 700 \times \left[P\right] + 400 \times \left[Al\right] + 400 \times \left[Ti\right] + 104 \times \left[V\right] - 11 \\ \times \left[Cr\right] + 31.5 \times \left[Mo\right] - 20 \times \left[Cu\right] - 15.2 \times \left[Ni\right]\end{matrix}$ $\begin{matrix} Ms point \left(°C\right) \\ = 550 - 361 \times \left[C\right] - 39 \times \left[Mn\right] - 10 \times \left[Cu\right] - 17 \times \left[Ni\right] - 20 \times \left[Cr\right] - 5 \times \left[Mo\right] + 30 \times \left[Al\right]\end{matrix}$ $Bs point \left(°C\right) = 830 - 270 \times \left[C\right] - 90 \times \left[Mn\right] - 37 \times \left[Ni\right] - 70 \times \left[Cr\right] - 83 \times \left[Mo\right]$
wherein [C], [Si], [Mn], [P], [Al], [Ti], [V], [Cr], [Mo], [Cu] and [Ni] represent the content (mass%) of C, Si, Mn, P, Al, Ti, V, Cr, Mo, Cu and Ni respectively. Also, when the element shown in each term of the formulae (2)-(5) above is not contained, calculation is done assuming that the term is null.

Treatment (1): The hot-rolled steel sheet was cold-rolled (sheet thickness: 1.6 mm).

Treatment (2): The hot-rolled steel sheet was cold-rolled (sheet thickness: 1.6 mm), was heated thereafter to 860°C simulating continuous annealing, was cooled thereafter to 400°C with the average cooling rate of 30°C/s, and was held.

Treatment (3): The hot-rolled steel sheet was cold-rolled (sheet thickness: 1.6 mm), was heated thereafter to 860°C simulating continuous hot dip galvanizing line, was cooled thereafter to 400°C with the average cooling rate of 30°C/s, was held, was thereafter heated further by (500°C×10 s), and was cooled thereafter.

**[Table 3]**

| Steel No. | Steel sheet manufacturing condition | | | | |
|---|---|---|---|---|---|
| | Heating temperature (°C) | Finish rolling temperature (°C) | Average cooling rate of finish rolling temperature - winding temperature (°C/s) | Winding temperature (°C) | Remarks |
| 1 | 1200 | 950 | 30 | 200 | - |
| 2 | 1200 | 950 | 30 | 200 | - |
| 3 | 1200 | 950 | 30 | 200 | - |
| 4 | 1200 | 950 | 30 | 200 | - |
| 5 | 1200 | 950 | 30 | 200 | - |
| 6 | 1200 | 820 | 30 | 200 | - |
| 7 | 1200 | 950 | 10 | 200 | - |
| 6 | 1200 | 950 | 30 | 400 | - |
| 9 | 1200 | 950 | 30 | 580 | |
| 10 | 1200 | 950 | 30 | 400 | Treatment (1) |
| 11 | 1200 | 950 | 30 | 400 | Treatment (2) |
| 12 | 1200 | 950 | 30 | 400 | Treatment (3) |
| 13 | 1200 | 950 | 30 | 200 | - |
| 14 | 1200 | 950 | 30 | 200 | - |
| 15 | 1200 | 950 | 30 | 200 | - |
| 16 | 1200 | 950 | 30 | 200 | - |
| 17 | 1200 | 950 | 30 | 200 | - |
| 18 | 1200 | 950 | 30 | 200 | - |
| 19 | 1200 | 950 | 30 | 200 | - |
| 20 | 1200 | 950 | 30 | 200 | - |
| 21 | 1200 | 950 | 30 | 200 | - |
| 22 | 1200 | 950 | 30 | 200 | - |
| 23 | 1200 | 950 | 30 | 200 | - |
| 24 | 1200 | 950 | 30 | 200 | - |
| 25 | 1200 | 950 | 30 | 200 | - |
| 26 | 1200 | 950 | 30 | 200 | - |
| 27 | 1200 | 950 | 30 | 200 | - |
| 28 | 1200 | 950 | 30 | 200 | - |
| 29 | 1200 | 950 | 30 | 200 | - |
| 30 | 1200 | 950 | 30 | 200 | - |
| 31 | 1200 | 950 | 30 | 200 | - |
| 32 | 1200 | 950 | 30 | 200 | - |

With respect to the steel sheet obtained, analysis of the precipitation state of Ti and observation of the metal microstructure (the fraction of each microstructure) were executed by the procedure described below. The result is shown in Tables 4, 5 below along with the calculated value of 0.5×[total Ti amount(mass%)-3.4[N]] (shown as 0.5×(total Ti amount-3.4[N])).

### [Analysis of precipitation state of Ti of steel sheet]

An extraction replica sample was prepared, and a transmission electron microscope image (magnifications: 100,000 times) of Ti-containing precipitates was photographed using a transmission electron microscope (TEM). At this time, by composition analysis of the precipitates using an energy dispersion type X-ray spectrometer (EDX), Ti-containing precipitates were identified. The area of the Ti-containing precipitates of at least 100 pieces was measured by image analysis, those having the equivalent circle diameter of 30 nm or less were extracted, and the average value thereof was made the size of the precipitates. Also, in the table, the size is shown as "average equivalent circle diameter of Ti-containing precipitates". Further, with respect to precipitated Ti amount (mass%)-3.4[N] (the Ti amount present as the precipitates), extraction residue analysis (in extraction treatment, the precipitates coagulate, and fine precipitates also can be measured) was executed using a mesh with mesh diameter: 0.1 µm, and precipitated Ti amount (mass%)-3.4[N] (expressed as "precipitated Ti amount-3.4[N]" in Tables 4, 5) was obtained. Also, when the Ti-containing precipitates partly contained V and Nb, the contents of these precipitates were also measured.

### [Observation of metal microstructure (fraction of each microstructure)]

(1) With respect to the microstructure of martensite and bainite in the steel sheet, the steel sheet was corroded by nital, martensite and bainite were distinguished from each other by SEM observation (magnifications: 1,000 times or 2,000 times), and each fraction (area ratio) was obtained.
(2) The retained austenite fraction in the steel sheet was measured by X-ray diffraction method after the steel sheet was ground up to 1/4 thickness thereof and was thereafter subjected to chemical polishing (for example, ISJJ Int. Vol. 33. (1933), No. 7, P.776).

**[Table 4]**

| Steel No. | Steel sheet for press forming use | | | | | |
|---|---|---|---|---|---|---|
| | Precipitated Ti amount-3.4[N] (mass%) | 0.5 × (total Ti amount-3.4[N]) (mass%) | Average equivalent circle diameter of Ti-containing precipitates (nm) | Fraction of martensite (area%) | Fraction of bainite (area%) | Others |
| 1 | 0.003 | 0.015 | 2.5 | 100 | 0 | - |
| 2 | 0.004 | 0.015 | 2.9 | 100 | 0 | - |
| 3 | 0.004 | 0.015 | 2.8 | 100 | 0 | - |
| 4 | 0.004 | 0.015 | 2.7 | 100 | 0 | - |
| 5 | 0.001 | 0.003 | 2.3 | 100 | 0 | - |
| 6 | 0.023 | 0.015 | 3.8 | 100 | 0 | - |
| 7 | 0.004 | 0.015 | 2.4 | 0 | 65 | Ferrite : 35% |
| 8 | 0.004 | 0.015 | 2.1 | 12 | 88 | - |
| 9 | 0.020 | 0.015 | 2.0 | 0 | 40 | Ferrite : 30%, Pearlite : 30% |
| 10 | 0.003 | 0.015 | 2.2 | 10 | 90 | - |
| 11 | 0.004 | 0.015 | 2.7 | 10 | 90 | - |
| 12 | 0.004 | 0.015 | 2.5 | 10 | 90 | - |
| 13 | 0.003 | 0.015 | 2.0 | 100 | 0 | - |
| 14 | 0.005 | 0.015 | 2.6 | 100 | 0 | |
| 15 | 0.005 | 0.015 | 2.2 | 100 | 0 | - |
| 16 | 0.004 | 0.015 | 2.6 | 90 | 0 | Retained austenite 10% |

**[Table 5]**

| Steel No. | Steel sheet for press forming use | | | | | |
|---|---|---|---|---|---|---|
| | Precipitated Ti amount-3.4[N] (mass%) | 0.5 × (total Ti amount-3.4[N]) (mass%) | Average equivalent circle diameter of Ti-containing precipitates (nm) | Fraction of martensite (area%) | Fraction of bainite (area%) | Others |
| 17 | 0.005 | 0.015 | 2.7 | 80 | 0 | Retained austenite 20% |
| 18 | 0.003 | 0.015 | 2.2 | 60 | 0 | Retained austenite 40% |
| 19 | 0.005 | 0.015 | 2.0 | 100 | 0 | - |
| 20 | 0.003 | 0.015 | 3.0 | 100 | 0 | - |
| 21 | 0.032 | 0.043 | 2.1 | 100 | 0 | - |
| 22 | 0.130 | 0.093 | 12.0 | 100 | 0 | - |
| 23 | 0.005 | 0.015 | 2.6 | 100 | 0 | - |
| 24 | 0.003 | 0.015 | 2.6 | 100 | 0 | - |
| 25 | 0.003 | 0.015 | 2.8 | 100 | 0 | - |
| 26 | 0.003 | 0.015 | 2.6 | 100 | 0 | - |
| 27 | 0.003 | 0.015 | 2.4 | 100 | 0 | - |
| 28 | 0.003 | 0.015 | 2.8 | 100 | 0 | - |
| 29 | 0.003 | 0.015 | 2.7 | 100 | 0 | - |
| 30 | 0.003 | 0.015 | 2.6 | 100 | 0 | - |
| 31 | 0.003 | 0.015 | 2.5 | 100 | 0 | - |
| 32 | 0.003 | 0.015 | 2.7 | 100 | 0 | - |

Each steel sheet described above (1.6 mm^{t}×150 mm×200 mm) (with respect to those other than the treatment of (1)-(3) described above, the thickness was adjusted to 1.6 mm by hot rolling) was heated to a predetermined temperature in a heating furnace, and was thereafter subjected to press forming and cooling treatment using the tool (Fig. 1 above) of a hat shape to obtain the formed product. The press forming conditions (heating temperature, average cooling rate, and rapid cooling finishing temperature in press forming) are shown in Table 6 below.

**[Table 6]**

| Steel No. | Press forming condition | | |
|---|---|---|---|
| | Heating temperature (°C) | Average cooling rate (°C/s) | Rapid cooling finishing temperature (°C) |
| 1 | 810 | 40 | 300 |
| 2 | 810 | 40 | 300 |
| 3 | 760 | 40 | 300 |
| 4 | 770 | 40 | 300 |
| 5 | 800 | 40 | 300 |
| 6 | 810 | 40 | 300 |
| 7 | 810 | 40 | 300 |
| 8 | 810 | 40 | 300 |
| 9 | 810 | 40 | 300 |
| 10 | 810 | 40 | 300 |
| 11 | 810 | 40 | 300 |
| 12 | 810 | 40 | 300 |
| 13 | 810 | 5 | 300 |
| 14 | 810 | 40 | 600 |
| 15 | 830 | 40 | 300 |
| 16 | 790 | 40 | 300 |
| 17 | 790 | 40 | 300 |
| 18 | 770 | 40 | 300 |
| 19 | 820 | 40 | 300 |
| 20 | 780 | 40 | 300 |
| 21 | 830 | 40 | 300 |
| 22 | 840 | 40 | 300 |
| 23 | 830 | 40 | 300 |
| 24 | 820 | 40 | 300 |
| 25 | 810 | 40 | 300 |
| 26 | 810 | 40 | 300 |
| 27 | 800 | 40 | 300 |
| 28 | 810 | 40 | 300 |
| 29 | 810 | 40 | 300 |
| 30 | 810 | 40 | 300 |
| 31 | 800 | 40 | 300 |
| 32 | 810 | 40 | 300 |

With respect to the formed product obtained, tensile strength (TS), elongation (total elongation EL), observation of the metal microstructure (the fraction of each microstructure), and hardness drop amount after heat treatment were measured by methods described below.

### [Measurement of tensile strength (TS) and elongation (total elongation EL)]

The tensile test was executed using JIS No. 5 test specimen, and the tensile strength (TS) and the elongation (EL) were measured. At this time, the strain rate of the tensile test was made 10 mm/s. In the present invention, the case 780-1,270 MPa of the tensile strength (TS) and 20% or more of the elongation (EL) were satisfied and the strength-elongation balance (TS×EL) was 20,000 (MPa· %) or more was evaluated to have passed.

### [Observation of metal microstructure (fraction of each microstructure)]

(1) With respect to the microstructure of annealed martensite, bainite and annealed bainite in the steel sheet, the steel sheet was corroded by nital, annealed martensite, bainite and annealed bainite were distinguished from each other by SEM observation (magnifications: 1,000 times or 2,000 times), and each fraction (area ratio) was obtained.
(2) The retained austenite fraction in the steel sheet was measured by X-ray diffraction method after the steel sheet was ground up to 1/4 thickness thereof and was thereafter subjected to chemical polishing (for example, ISJJ Int. Vol. 33. (1933), No. 7, P.776).
(3) With respect to the fraction of martensite as quenched, the steel sheet was LePera-corroded, the area ratio of the white contrast was measured as the mixture microstructure of martensite as quenched and retained austenite, the retained austenite fraction obtained by X-ray diffraction was deducted therefrom, and the fraction of martensite as quenched was calculated.

### [Hardness drop amount after heat treatment]

As the thermal hysteresis based on spot welding, heating was executed to 700°C with the average heating rate of 50°C/s using a heat treatment simulator, cooling was thereafter executed with the average cooling rate of 50°C/s, and the hardness drop amount (ΔHv) relative to the original hardness (Vickers hardness) was measured. When the hardness drop amount (ΔHv) was 50Hv or less, the softening prevention property in the HAZ was determined to be excellent.

The observation results (fraction of each microstructure, precipitated Ti amount-3.4[N]) of the metal microstructure are shown in Tables 7, 8 below. Also, the mechanical properties (tensile strength TS, elongation EL, TS×EL, and hardness drop amount ΔHv) of the formed product are shown in Table 9 below. Further, although the value of precipitated Ti amount-3.4[N] in the formed product is slightly different compared to the value of precipitated Ti amount-3.4[N] in the steel sheet for press forming use, this is a measurement error.

**[Table 7]**

| Steel No. | Metal microstructure of formed product | | | | | |
|---|---|---|---|---|---|---|
| | Fraction of annealed martensite and/or annealed bainite (area%) | Fraction of martensite as quenched (area%) | Fraction of retained austenite (area%) | Average equivalent circle diameter of Ti-containing precipitates (nm) | Precipitated Ti amount-3.4[N] (mass%) | Others |
| 1 | 70 | 23 | 7 | 2.1 | 0.005 | - |
| 2 | 70 | 23 | 7 | 2.5 | 0.005 | Ferrite 3% |
| 3 | 70 | 30 | 0 | 2.4 | 0.009 | - |
| 4 | 70 | 25 | 5 | 2.5 | 0.008 | - |
| 5 | 70 | 23 | 7 | 2.3 | 0.001 | - |
| 6 | 70 | 23 | 7 | 13 | 0.025 | - |
| 7 | 50 | 8 | 7 | 2.2 | 0.005 | Ferrite 35% |
| 8 | 70 | 23 | 4 | 2.9 | 0.007 | - |
| 9 | 70 | 23 | 7 | 3.2 | 0.031 | - |
| 10 | 70 | 23 | 7 | 2.6 | 0.010 | - |
| 11 | 70 | 23 | 7 | 2.0 | 0.010 | - |
| 12 | 70 | 23 | 7 | 2.8 | 0.010 | - |
| 13 | 70 | 0 | 0 | 2.3 | 0.005 | Bainite 25%, Pearlite 5% |
| 14 | 70 | 23 | 7 | 2.2 | 0.008 | - |
| 15 | 70 | 23 | 9 | 2.4 | 0.005 | - |
| 16 | 60 | 29 | 11 | 2.4 | 0.010 | - |

**[Table 8]**

| Steel No. | Metal microstructure of formed product | | | | | |
|---|---|---|---|---|---|---|
| | Fraction of annealed martensite and/or annealed bainite (area%) | Fraction of martensite as quenched (area%) | Fraction of retained austenite (area%) | Average equivalent circle diameter of Ti-containing precipitates (nm) | Precipitated Ti amount-3.4[N] (mass%) | Others |
| 17 | 55 | 32 | 13 | 2.3 | 0.005 | - |
| 18 | 16 | 62 | 22 | 2.1 | 0.006 | - |
| 19 | 70 | 25 | 5 | 2.3 | 0.008 | - |
| 20 | 70 | 21 | 9 | 2.5 | 0.010 | - |
| 21 | 70 | 23 | 7 | 2.7 | 0.040 | - |
| 22 | 70 | 23 | 7 | 12.0 | 0.180 | - |
| 23 | 70 | 23 | 7 | 2.0 | 0.009 | - |
| 24 | 70 | 23 | 7 | 2.6 | 0.010 | - |
| 25 | 70 | 23 | 7 | 2.8 | 0.008 | - |
| 26 | 70 | 23 | 7 | 2.1 | 0.006 | - |
| 27 | 70 | 23 | 7 | 3.0 | 0.009 | - |
| 28 | 70 | 23 | 7 | 2.7 | 0.006 | - |
| 29 | 70 | 24 | 6 | 2.7 | 0.008 | - |
| 30 | 70 | 22 | 8 | 2.5 | 0.007 | - |
| 31 | 70 | 23 | 7 | 2.7 | 0.008 | - |
| 32 | 70 | 24 | 6 | 2.8 | 0.007 | - |

**[Table 9]**

| Steel No. | Mechanical properties of formed product | | | |
|---|---|---|---|---|
| | Tensile strength TS (MPa) | Elongation EL (%) | TS × EL (MPa·%) | Hardness drop amount ΔHv (Hv) |
| 1 | 1016 | 21.6 | 21919 | 21 |
| 2 | 1027 | 20.9 | 21461 | 22 |
| 3 | 1050 | 13.0 | 13650 | 23 |
| 4 | 983 | 22.3 | 21906 | 22 |
| 5 | 1022 | 22.4 | 22894 | 26 |
| 6 | 1524 | 10.3 | 15697 | 52 |
| 7 | 721 | 19.4 | 13987 | 22 |
| 8 | 1011 | 21.8 | 22040 | 22 |
| 9 | 1053 | 20.8 | 21908 | 62 |
| 10 | 1064 | 21.3 | 22628 | 22 |
| 11 | 1048 | 20.2 | 21178 | 21 |
| 12 | 1061 | 21.2 | 22535 | 21 |
| 13 | 876 | 16.2 | 14191 | 22 |
| 14 | 1053 | 20.1 | 21120 | 22 |
| 15 | 1047 | 23.0 | 24112 | 22 |
| 16 | 1192 | 20.3 | 24188 | 21 |
| 17 | 1260 | 21.4 | 26955 | 21 |
| 18 | 1321 | 10.2 | 13474 | 22 |
| 19 | 1016 | 23.6 | 23984 | 22 |
| 20 | 1054 | 22.6 | 23811 | 21 |
| 21 | 1047 | 22.6 | 23678 | 28 |
| 22 | 1071 | 16.4 | 17564 | 51 |
| 23 | 1060 | 22.8 | 24143 | 22 |
| 24 | 1052 | 23.1 | 24343 | 21 |
| 25 | 1045 | 22.3 | 23283 | 22 |
| 26 | 1042 | 23.7 | 24648 | 21 |
| 27 | 1062 | 22.0 | 23409 | 22 |
| 28 | 1051 | 22.5 | 23603 | 22 |
| 29 | 1020 | 22.6 | 23052 | 22 |
| 30 | 1041 | 22.5 | 23423 | 21 |
| 31 | 1033 | 23.1 | 23862 | 21 |
| 32 | 1042 | 22.7 | 23653 | 22 |

From these results, following consideration can be made. Those of the steel Nos. 1, 2, 4, 5, 8, 10-12, 14-17, 19-21, 23-32 are examples fulfilling the requirements stipulated in the present invention, and it is known that components excellent in strength-elongation balance and excellent in softening prevention property have been obtained.

On the other hand, those of the steel Nos. 3, 6, 7, 9, 13, 18, 22 are the comparative examples not satisfying any of the requirements stipulated in the present invention, and any of the properties is deteriorated. That is, that of the steel No. 3 uses a steel sheet with low Si content, the fraction of retained austenite in the formed product is not secured, the elongation is not enough, and the strength-elongation balance is deteriorated. In that of the steel No. 6, the finish rolling temperature in manufacturing the steel sheet is low, the relationship of the formula (1) is not fulfilled in either stage of the steel sheet for hot pressing use and the formed product, the elongation is not enough to deteriorate the strength-elongation balance, and the softening prevention property is also deteriorated.

In that of the steel No. 7, the average cooling rate from the finish rolling temperature to winding in manufacturing the steel sheet is low, ferrite is formed in the stage of the formed product and the fraction of martensite as quenched cannot be secured, the strength and elongation drop, and the strength-elongation balance (TS×EL) is deteriorated. In that of the steel No. 9, the winding temperature in manufacturing the steel sheet is high, the precipitated Ti amount is excessive in the stage of the steel sheet for hot pressing use, and, when press forming is executed using such a steel sheet, even if the forming condition is appropriate, the precipitated Ti amount is excessive also in the formed product, and the softening prevention property is also deteriorated.

In that of the steel No. 13, the cooling rate in press forming is slow, bainite and pearlite are formed in the stage of the formed product and the fraction of martensite as quenched cannot be secured, the strength and elongation drop, and the strength-elongation balance (TS×EL) is deteriorated. In that of the steel No. 18, the steel sheet with excessive C content is used, the fraction of martensite of the steel sheet is low, the heating temperature in press forming is high, the fraction of martensite and/or annealed bainite in the formed product cannot be secured, the strength becomes high, and only low elongation EL is obtained (the strength-elongation balance (TS×EL) is also deteriorated). In that of the steel No. 22, the steel sheet with excessive Ti content is used, the strength-elongation balance (TS×EL) is deteriorated, and the softening prevention property is also deteriorated.

### [Example 2]

Steel (steel Nos. 33-37) having the chemical component composition shown in Table 10 below was molten in vacuum, was made a slab for experiment, was thereafter hot-rolled, and was thereafter cooled and wound (sheet thickness: 3.0 mm). The manufacturing condition for the steel sheet at that time is shown in Table 11 below.

**[Table 10]**

| Steel No. | Chemical component composition* (mass%) | | | | | | | | | | | | | | | Ac₃-20°C(°C) | Ac₁+20°C(°) | Bs-100°C(°C) | Ms point (°C) |
|---|---|---|---|---|---|---|---|---|---|---|---|---|---|---|---|---|---|---|---|
| | C | Si | Mn | P | S | Al | B | Ti | N | V | Nb | Cu | Ni | Cr | Mo | | | | |
| 33 | 0.220 | 1.20 | 1.20 | 0.0050 | 0.0020 | 0.030 | 0.0020 | 0.044 | 0.0040 | - | - | - | - | 0.20 | - | 843 | 768 | 549 | 421 |
| 34 | 0.220 | 1.20 | 1.20 | 0.0050 | 0.0020 | 0.030 | 0.0020 | 0.044 | 0.0040 | - | - | - | - | 0.20 | - | 843 | 768 | 549 | 421 |
| 35 | 0.350 | 1.20 | 1.20 | 0.0050 | 0.0020 | 0.030 | 0.0020 | 0.044 | 0.0040 | - | - | - | - | 0.20 | - | 818 | 768 | 514 | 374 |
| 36 | 0.220 | 1.20 | 1.20 | 0.0050 | 0.0020 | 0.030 | 0.0020 | 0.044 | 0.0040 | - | - | - | - | 0.20 | - | 843 | 768 | 549 | 421 |
| 37 | 0.220 | 1.20 | 1.20 | 0.0050 | 0.0020 | 0.030 | 0.0020 | 0.044 | 0.0040 | - | - | - | - | - | - | 845 | 765 | 563 | 425 |

| | | | | | | | | | | | | | | | | | | | |
|---|---|---|---|---|---|---|---|---|---|---|---|---|---|---|---|---|---|---|---|
| *The remainder: iron and inevitable impurities other than P, S, N. | | | | | | | | | | | | | | | | | | | |

**[Table 11]**

| Steel No: | Steel sheet manufacturing condition | | | | |
|---|---|---|---|---|---|
| | Heating temperature (°C) | Finish rolling temperature (°C) | Average cooling rate of finish rolling temperature - winding temperature (°C/s) | Winding temperature (°C) | Remarks |
| 33 | 1200 | 950 | 30 | 200 | - |
| 34 | 1200 | 950 | 30 | 200 | - |
| 35 | 1200 | 950 | 30 | 200 | - |
| 36 | 1200 | 950 | 30 | 200 | Treatment (1) |
| 37 | 1200 | 950 | 30 | 200 | - |

With respect to the steel sheet obtained, analysis of the precipitation state of Ti-containing precipitates and observation of the metal microstructure (the fraction of each microstructure) were executed similarly to Example 1. The result is shown in Table 12 below.

**[Table 12]**

| Steel No. | Steel sheet for press forming use | | | | | |
|---|---|---|---|---|---|---|
| | Precipitated Ti amount-3.4[N] (mass%) | 0.5 × (total Ti amount-3.4[N]) (mass%) | Average equivalent circle diameter of Ti-containing precipitates (nm) | Fraction of martensite (area%) | Fraction of bainite (area%) | Others |
| 33 | 0.002 | 0.015 | 2.7 | 100 | 0 | - |
| 34 | 0.003 | 0.015 | 2.9 | 100 | 0 | - |
| 35 | 0.004 | 0.015 | 2.3 | 90 | 0 | Retained austenite 10% |
| 36 | 0.001 | 0.015 | 3.0 | 100 | 0 | - |
| 37 | 0.002 | 0.015 | 2.5 | 100 | 0 | - |

Each steel sheet described above (3.0 mm^{t}×150 mmx200 mm) was heated to a predetermined temperature in a heating furnace, and was subjected thereafter to press forming and cooling treatment using the tool (Fig. 1 above) of a hat shape to obtain the formed product. At this time, the steel sheet was put in an infrared furnace and the portion intended to be high-strengthened (the steel sheet portion corresponding to the first region) was configured so that infrared rays directly hit so as to allow high temperature heating, whereas the portion intended to be low-strengthened (the steel sheet portion corresponding to the second region) was shielded with a cover so that a part of the infrared rays was blocked so as to allow low temperature heating, and thereby the heating temperature was differentiated. Therefore, the formed product has the regions with different strength within a single component. The press forming conditions (heating temperature, average cooling rate, and rapid cooling finishing temperature of each region in press forming) are shown in Table 13 below.

**[Table 13]**

| Steel No. | Region | Press forming condition | | |
|---|---|---|---|---|
| | | Heating temperature (°C) | Average cooling rate (°C/s) | Rapid cooling finishing temperature (°C) |
| 33 | Low strength side | 810 | 40 | 300 |
| | High strength side | 920 | 40 | 300 |
| 34 | Low strength side | 800 | 40 | 300 |
| | High strength side | 840 | 40 | 300 |
| 35 | Low strength side | 800 | 40 | 300 |
| | High strength side | 920 | 40 | 300 |
| 36 | Low strength side | 790 | 40 | 300 |
| | High strength side | 920 | 40 | 300 |
| 37 | Low strength side | 810 | 40 | 300 |
| | High strength side | 920 | 40 | 300 |

With respect to the formed product obtained, tensile strength (TS), elongation (total elongation EL), and observation of the metal microstructure (the fraction of each microstructure) in each region were obtained similarly to Example 1.

The observation results (fraction of each microstructure) of the metal microstructure are shown in Table 14 below. Also, the mechanical properties (tensile strength TS, elongation EL, TS×EL, and hardness drop amount) of the formed product are shown in Table 15 below.

Further, the case 1,470 MPa or more of the tensile strength (TS) and 8% or more of the elongation (EL) on the high strength side were fulfilled and the strength-elongation balance (TS×EL) was 14,000 (MPa· %) or more was evaluated to have passed (the evaluation criteria of the low strength side are same to those of Example 1).

**[Table 14]**

| Steel No. | Region | Metal microstructure of formed product | | | | | |
|---|---|---|---|---|---|---|---|
| | | Fraction of annealed martensite and/or annealed bainite (area%) | Fraction of martensite as quenched (area%) | Fraction of retained austenite (area%) | Average equivalent circle diameter of Ti-containing precipitates (nm) | Precipitated Ti amount-3.4[N] (mass%) | Others |
| 33 | Low strength side | 70 | 23 | 7 | 6.2 | 0.008 | - |
| | High strength side | 0 | 94 | 6 | 2.5 | 0.005 | - |
| 34 | Low strength side | 70 | 23 | 7 | 6.0 | 0.007 | - |
| | High strength side | 0 | 61 | 6 | 2.3 | 0.008 | Ferrite 33% |
| 35 | Low strength side | 60 | 29 | 11 | 6.0 | 0.009 | - |
| | High strength side | 0 | 95 | 5 | 2.4 | 0.008 | - |
| 36 | Low strength side | 70 | 23 | 7 | 4.0 | 0.005 | - |
| | High strength side | 0 | 94 | 6 | 2.9 | 0.007 | - |
| 37 | Low strength side | 70 | 24 | 6 | 5.8 | 0.009 | - |
| | High strength side | 0 | 94 | 6 | 2.7 | 0.008 | - |

**[Table 15]**

| Steel No. | Region | Mechanical properties of formed product | | | |
|---|---|---|---|---|---|
| | | Tensile strength TS (MPa) | Elongation EL (%) | TS × EL (MPa·%) | Hardness drop amount ΔHv(Hv) |
| 33 | Low strength side | 1010 | 21.4 | 21586 | 30 |
| | High strength side | 1511 | 10.1 | 15261 | 45 |
| 34 | Low strength side | 1014 | 21.8 | 22117 | 30 |
| | High strength side | 1278 | 12.1 | 15464 | 42 |
| 35 | Low strength side | 1192 | 21.6 | 25740 | 30 |
| | High strength side | 1820 | 9.7 | 17654 | 50 |
| 36 | Low strength side | 1066 | 21.9 | 23345 | 30 |
| | High strength side | 1499 | 10.1 | 15140 | 43 |
| 37 | Low strength side | 1007 | 20.3 | 20442 | 30 |
| | High strength side | 1501 | 10.8 | 16211 | 45 |

From this result, following consideration can be made. Those of the steel Nos. 33, 35-37 are examples fulfilling the requirements stipulated in the present invention, and it is known that components excellent in strength-elongation balance in each region have been obtained. On the other hand, in that of the steel No. 34, the heating temperature in press forming is low, and the strength on the high strength side drops (the strength difference relative to the low strength side is less than 300 MPa).

Although the present invention has been described in detail and referring to specific embodiments, it is obvious for a person with an ordinary skill in the art that various alterations and amendments can be effected without departing from the spirit and the range of the present invention.

The present application is based on Japanese Patent Application (JP-A-No. 2012-053845) applied on March 9, 2012, and the contents thereof are hereby incorporated by reference.

### [Industrial Applicability]

The steel sheet for hot pressing use of the present invention is suitable to structural components of an automobile.

### [Reference Signs List]

1... paunch
2...die
3...blank holder
4...steel sheet (blank)

## Claims

1. A steel sheet for hot pressing use comprising:
C: 0.15-0.5% (means mass%, hereinafter the same with respect to the chemical component composition);
Si: 0.2-3%;
Mn: 0.5-3%;
P: 0.05% or less (exclusive of 0%);
S: 0.05% or less (exclusive of 0%);
Al: 0.01-1%;
B: 0.0002-0.01%;
Ti: 3.4[N]+0.002% or more and 3.4[N]+0.1% or less ([N] expresses N content (mass%)), and
N: 0.001-0.01% respectively, with the remainder consisting of iron and inevitable impurities, wherein
some of Ti-containing precipitates contained in the steel sheet, each of which having an equivalent circle diameter of 30 nm or less, have an average equivalent circle diameter of 6 nm or less, the precipitated Ti amount and the total Ti amount in the steel fulfill the relationship represented by formula (1) shown below, and the sum total of the fraction of bainite and the fraction of martensite in the metal microstructure is 80 area% or more. $Precipitated Ti amount \left(mass%\right) - 3.4 \left[N\right] \leq 0.5 \times \left[\left(total Ti amount \left(mass%\right)\right)-3.4\left[N\right]\right]$ (In the formula (1), [N] represents the content (mass%) of N in the steel.)

2. The steel sheet for hot pressing use according to claim 1 further comprising at least one of (a)-(c) below as other elements:
(a) at least one element selected from the group consisting of V, Nb and Zr by 0.1% or less (exclusive of 0%) in total;
(b) at least one element selected from the group consisting of Cu, Ni, Cr and Mo by 1% or less (exclusive of 0%) in total; and
(c) at least one element selected from the group consisting of Mg, Ca and REM by 0.01% or less (exclusive of 0%) in total.

3. A method for manufacturing a press-formed product comprising the steps of:
heating the steel sheet for hot pressing use according to claim 1 or 2 to a temperature of Ac₁ transformation point+20°C or above and Ac₃ transformation point-20°C or below;
thereafter starting press-forming of the steel sheet; and
holding the steel sheet at the bottom dead point and executing cooling to a temperature or below, the temperature being lower than the bainite transformation starting temperature Bs by 100°C, while securing the average cooling rate of 20°C/s or more within a tool.

4. A press-formed product of a steel sheet having the chemical component composition according to claim 1 or 2, wherein metal microstructure within the press-formed product comprises retained austenite: 3-20 area%, annealed martensite and/or annealed bainite: 30-87 area%, and martensite as quenched: 10-67 area%, some of Ti-containing precipitates contained in pressed steel, each of which having an equivalent circle diameter of 30 nm or less, have an average equivalent circle diameter of 10 nm or less, and the amount of precipitated Ti and the total amount of Ti in the formed product fulfill the relationship represented by the formula (1) shown below. $Precipitated Ti amount \left(mass%\right) - 3.4 \left[N\right] \leq 0.5 \times \left[\left(total Ti amount \left(mass%\right)\right)-3.4\left[N\right]\right]$ (In the formula (1), [N] represents the content (mass%) of N in the steel.)

5. A method for manufacturing a press-formed product comprising the steps of:
using the steel sheet for hot pressing use according to claim 1 or 2;
dividing a heating region of the steel sheet into at least two regions;
heating one region thereof to a temperature of Ac₃ transformation point or above and 950°C or below;
heating another region to a temperature of Ac₁ transformation point+20°C or above and Ac₃ transformation point-20°C or below;
thereafter starting press forming of the both regions; and
holding the both regions at the bottom dead point and executing cooling to a temperature of martensite transformation starting temperature Ms or below while securing the average cooling rate of 20°C/s or more within a tool.

6. A press-formed product of a steel sheet having the chemical component composition according to claim 1 or 2, wherein
the press-formed product includes a first region whose metal microstructure comprises retained austenite: 3-20 area% and martensite as quenched: 80 area% or more, and a second region whose metal microstructure comprises retained austenite: 3-20 area%, annealed martensite and/or annealed bainite: 30-87 area%; and martensite as quenched: 10-67 area%,
some of Ti-containing precipitates contained in steel of the second region, each of which having an equivalent circle diameter of 30 nm or less, have an average equivalent circle diameter of 10 nm or less, and
the precipitated Ti amount and the total Ti amount in the formed product fulfill the relationship represented by the formula (1) shown below. $Precipitated Ti amount \left(mass%\right) - 3.4 \left[N\right] \leq 0.5 \times \left[\left(total Ti amount \left(mass%\right)\right)-3.4\left[N\right]\right]$ (In the formula (1), [N] represents the content (mass%) of N in the steel.)
